

## UNITED STATES PATENT OFFICE

2,365,084

## BENEFICIATION OF ACIDIC MINERALS

David W. Jayne, Jr., Old Greenwich, Harold M. Day, Cos Cob, and Elmer W. Gieseke, Stamford, Conn., assignors to American Cyanamid Company, New York, N. Y., a corporation of Maine

No Drawing. Application March 31, 1942,  
Serial No. 437,037

8 Claims. (Cl. 209—166)

The present invention relates to mineral concentration and more particularly relates to the use of a new class of reagents for selectively separating acidic minerals from other ore constituents.

Still more particularly, the present invention relates to the use of higher alkyl substituted guanidines, biguanides, guanylthioureas, guanylureas, and salts thereof, as promoters or collectors for acidic minerals in froth flotation, film flotation, stratification, agglomeration, tabling and related mineral separation processes. While the present invention is not limited to any particular ore concentrating process utilizing differential surface wettability principles or to any particular ore, its most important field of usefulness is in connection with froth flotation processes of separating silica or silicate minerals, such as mica, from non-metallic ores including limestone, bauxite, barytes ilmenite, calcite, and the like, and especially phosphate minerals wherein the silicious gangue is floated away from the phosphate minerals.

In accordance with this invention natural ores or artificial materials comprising a mixture of acidic minerals with other mineral constituents are subjected to a separation or concentration process in the presence of a promoter for the acidic ore minerals, said promoter being a higher alkyl derivative of guanidine, biguanide, guanylthiourea, guanylurea, or salt thereof.

The reagents of the present invention are effective promoters or collectors for negatively charged or acidic ore materials generally and said acidic material may either be worthless gangue or valuable ore constituents. The most important uses are, however, in connection with the froth flotation of silica from non-metallic ores in which the silicious gangue may represent a minor proportion of the ore rather than metallic and sulfide ores in which the gangue usually represents the major proportion of the ore. Representative acidic ore materials are the feldspars, quartz, pyroxenes, the spinels, biotite, muscovite, clays, and the like.

The compounds that have been found to have a selective filming attraction for acidic ores and which are useful for carrying out this invention include broadly the higher alkyl substituted 5 guanidines, biguanides, guanylthioureas, and guanylureas and salts thereof. Compounds falling within this classification may be represented by the following formula:



in which R is an alkyl radical containing from 10 8 to 20 carbon atoms, R' is hydrogen or an alkyl radical containing from 8 to 20 carbon atoms and Y represents hydrogen, or a radical such as



20 and the salts of such compounds. An examination of the general formula shows that the compounds are all higher alkylated derivatives of guanidines, biguanides, guanylthioureas, guanylureas, and the like. We have found that while guanidine, 25 biguanide, guanylthiourea and guanylurea, themselves, have no promoter action for acidic ore materials, they can be converted into effective promoters by replacing at least one of the hydrogen on an amino nitrogen group with an aliphatic radical having from about 8 to about 20 carbon atoms. Further, we have found that effective 30 promoters are also obtained wherein both hydrogens on an amino group are replaced by alkyl radicals having from about 8 to 20 carbon atoms 35 to give the higher di-alkyl derivatives.

The compounds which we use in carrying out the process of the present invention may be prepared by any satisfactory method and the invention is not particularly concerned with their 40 method of preparation. These compounds may be conveniently prepared by reaction of a higher alkyl primary or secondary amine with the hydrohalide salt of lower S-alkyl pseudo-thiourea, pseudo-guanylthiourea, pseudo-monothiobiuret, 45 or pseudo-dithiobiuret to yield respectively the

alkyl guanidine, biguanide, guanylurea, or guanylthiourea hydrohalides; according to the following reactions:



in which R is an alkyl radical containing from 8 to 20 carbon atoms, R' is hydrogen or an alkyl radical containing from 8 to 20 carbon atoms, R'' is an alkyl radical containing from 1 to 3 carbon atoms, and X is a halogen radical.

The hydrohalides of the lower alkyl pseudo compounds used in the above reactions may be conveniently prepared by the action of a lower alkyl halide, such as ethyl iodide, on thiourea, guanylthiourea, monothiobiuret or dithiobiuret, respectively.

The higher alkyl guanidines may also be prepared by the reaction of cyanamide with the hydrochlorides of higher mono- or di-alkyl amines.

The higher alkyl biguanides may also be prepared by the reaction of dicyandiamide with the hydrochlorides of higher mono- or di-alkyl amines.

We do not limit ourselves to the use of these compounds prepared by any particular method, nor to the use of the hydrohalide salts of such compounds. The free base may be used, and we also include the use of other salts (such as acetate) produced from the free base.

Examples of representative compounds falling within the scope of our invention include the following: unsymmetrical di-octyl guanidine hydrobromide, cetyl guanidine hydroiodide, lauryl biguanide hydrochloride, tetradecyl guanylurea hydrobromide, and lauryl guanylthiourea hydrobromide.

By way of illustration the following processes show the preparation of an alkyl guanidine, biguanide, and guanylthiourea:

1. "Lorol" guanidine hydroiodide

23.2 grams of S-ethyl pseudo-thiourea hydro-

iodide and 20 grams of "Lorol" amine (technical mixture C<sub>8</sub>-C<sub>16</sub> primary aliphatic amines, averaging about C<sub>13</sub>) in 50 cc. of anhydrous ethanol was heated under reflux on a steam bath for 8 hours with evolution of ethyl mercaptan. The alcohol was then completely removed by distillation under reduced pressure. The product was a light-brown crystalline paste, soluble in water to give a "soapy" solution.

2. "Lorol" biguanide hydroiodide

Same procedure as 1 using 18.5 grams of S-ethyl pseudo-guanyl-thiourea hydroiodide and 13.5 grams of "Lorol" amine in 100 cc. of anhydrous ethanol. The product was similar to that obtained in 1.

3. "Lorol" guanylthiourea hydroiodide

Same procedure as 1 using 29.1 grams of S-ethyl pseudo-dithiobiuret hydroiodide and 20 grams of "Lorol" amine in 100 cc. of anhydrous ethanol. The product was a yellow paste, soluble in water to give a "soapy" solution.

The compounds mentioned heretofore and which are useful in carrying out our invention are usually homogeneous, viscous pastes which will combine with acids, such as formic, acetic, hydrochloric, hydrobromic, and the like, to yield salts which are soluble in water. They may be used in flotation processes in the form of these water soluble salts or the free base may be used provided satisfactory dispersion is obtained.

While, as stated heretofore, the present invention is not limited to the treatment of any particular ore material, it has been found to be well suited for froth flotation of silica from phosphate rock and is the preferred embodiment of the invention. In the processes of removing silica from phosphate rock, the conditions are such that practically complete removal of the silica must be accomplished in order to produce a salable phosphate material. It is therefore an advantage of this invention that our reagents not only effect satisfactory removal of the silica but are also economical in amounts used. The quantities required range from 0.2 pound per ton of ore depending upon the particular ore and the particular reagent. The invention is not, however, limited to such quantities.

The reagents of the present invention may be used alone or in mixtures with other promoters. They may likewise be used in conjunction with other cooperating materials such as conditioning reagents, oily or fat materials such as hydrocarbon oils, fatty acids, or fatty acid esters.

These new reagents are also adaptable for use in any of the ordinary concentrating processes such as film flotation, tabling, and particularly in froth flotation operations. The ore concentrating processes employed will depend upon the particular type or kind of ore which is being processed. For example, in connection with phosphate rock, relatively coarse phosphate bearing material, for example 28 mesh and larger, can be very economically concentrated by using these reagents in conjunction with a material such as fuel oil or pine oil and subjecting to concentration by the use of tables or by film flotation. The -28 phosphate rock material is best concentrated by means of froth flotation employing these improved silica promoters.

When the reagents of the present invention are employed as promoters in the froth flotation of silica from phosphate rock, which is the preferred embodiment thereof, the condition may be

varied in accordance with procedures known to those skilled in the art. The reagent may be employed in the form of aqueous solutions, emulsions, mixtures, or solutions in organic solvents, such as alcohol and the like. The reagent may be introduced into the ore pulp prior to the actual concentration operation. They may also be stage fed into the flotation circuit.

In its most important aspect the present invention is utilized for the treatment of non-metallic ore materials but it is to be understood that our reagents under proper conditions may be used advantageously for the treatment of metallic ore materials.

Other improved phosphate flotation features which are known may be utilized in connection with the present invention such as splitting the phosphate flotation feed into a plurality of size ranges and floating each size separately as described in the U. S. Patent No. 2,156,245, the very complete removal of the slime prior to flotation which is also an aid to better results as pointed out in the Erickson application, Serial No. 325,011 filed March 20, 1941, and the Mead and Maust application Serial No. 320,121 filed February 21, 1940, which describes a process for classifying and desliming phosphate flotation feed by means of a hindered settling classifier and which deslimed feed is well suited for treatment in accordance with this invention.

This invention will be further illustrated by the following specific tests which are illustrations of the preferred embodiments thereof, but is not to be strictly limited thereby.

Flotation tests as follows were made on a sample of Florida phosphate rock from the Old Colony Mine near Brewster. A fine flotation feed (-35 +200 mesh) was produced by scrubbing, polishing, and desliming until the ore material was substantially free of slimes.

Separate 600-gram samples of the deslimed flotation feed were diluted to 22% solids with water and transferred to a laboratory size Fagergren flotation machine. The particular reagent or reagent combination was then added and conditioned with the pulp for three seconds. Air was then admitted to the machine and the resulting concentrate froth was collected until the froth became barren. The flotation test products were then filtered, dried, weighed, and assayed. The metallurgical data obtained in these tests are presented in Table I.

Table I

| Test No. | Feed percent insol. | Concentrate |                |                      | Tailing     |                |                      | Reagents      | Lbs./ton of feed |
|----------|---------------------|-------------|----------------|----------------------|-------------|----------------|----------------------|---------------|------------------|
|          |                     | Percent wt. | Percent insol. | Dist. percent insol. | Percent wt. | Percent insol. | Dist. percent insol. |               |                  |
| 1.....   | 54.54               | 61.02       | 87.59          | 98.00                | 38.98       | 2.79           | 2.00                 | a.....        | 0.50             |
| 2.....   | 54.54               | 58.34       | 88.14          | 94.28                | 41.66       | 7.50           | 5.72                 | Pine oil..... | 0.12             |
| 3.....   | 54.54               | 59.70       | 87.87          | 96.19                | 40.80       | 6.17           | 3.81                 | b.....        | 0.50             |
|          |                     |             |                |                      |             |                |                      | Pine oil..... | 0.12             |
|          |                     |             |                |                      |             |                |                      | c.....        | 0.50             |
|          |                     |             |                |                      |             |                |                      | Pine oil..... | 0.12             |

*a* Lauryl guanidine hydroiodide.

*b* Lauryl biguanide hydroiodide.

*c* Lauryl guanylthiourea hydroiodide.

When rake classifier sands such as those produced from the tailings at the Valley Forge Cement Company plants are treated by flotation using our reagents, the alumina in the form of mica, is removed in part from the silicious material and a cement product is produced which has greatly improved properties.

In the treatment of iron ores we have found that our reagent may be employed in flotation processes for removing the silica therefrom and the tailings resulting from such processes are much higher in iron content than concentrates produced by the conventional soap flotation of the iron minerals.

What we claim is:

1. In the froth flotation process of separating acidic silicious gangue from non-metallic ore values, the step which comprises subjecting the ore to froth flotation in the presence of an effective amount of a product of the group consisting of those represented by the following formula:



in which R is an alkyl radical containing from 8 to 20 carbon atoms, R' is a member of the group consisting of hydrogen and an alkyl radical containing from 8 to 20 carbon atoms and Y is a member of the group consisting of hydrogen and



radicals, and salts of such compounds to effect a substantially complete separation of the ore values from the acidic silicious gangue thereby producing a tailing high in phosphate and relatively low in gangue.

2. In the froth flotation process of separating acidic silicious gangue from phosphate ore values, the step which comprises subjecting the ore to froth flotation in the presence of an effective amount of a product of the group consisting of those represented by the following formula:



in which R is an alkyl radical containing from 8 to 20 carbon atoms, R' is a member of the group consisting of hydrogen and an alkyl radical containing from 8 to 20 carbon atoms, and Y is a member of the group consisting of hydrogen and



radicals, and salts of such compounds to effect a substantially complete separation of the ore

values from the acidic silicious gangue thereby producing a tailing high in phosphate and relatively low in gangue.

3. In the froth flotation process of separating acidic silicious gangue from phosphate ore values, the step which comprises subjecting the ore to froth flotation in the presence of an effec-

tive amount of a product of the group consisting of those represented by the following formula:



in which R is an alkyl radical containing from 8 to 20 carbon atoms, R' is a member of the group consisting of hydrogen and an alkyl radical containing from 8 to 20 carbon atoms, and X is a halogen radical, and salts of such compounds to effect a substantially complete separation of the ore values from the acidic silicious gangue thereby producing a tailing high in phosphate and relatively low in gangue.

4. In the froth flotation process of separating acidic silicious gangue from phosphate ore values, the step which comprises subjecting the ore to froth flotation in the presence of an effective amount of a product of the group consisting of those represented by the following formula:



in which R is an alkyl radical containing from 8 to 20 carbon atoms, R' is a member of the group consisting of hydrogen and an alkyl radical containing from 8 to 20 carbon atoms, and X is a halogen radical, and salts of such compounds to effect a substantially complete separation of the ore values from the acidic silicious gangue thereby producing a tailing high in phosphate and relatively low in gangue.

5. In the froth flotation process of separating acidic silicious gangue from phosphate ore values, the step which comprises subjecting the ore to froth flotation in the presence of an effective amount of a product of the group consisting of those represented by the following formula:



in which R' is a member of the group consisting of hydrogen and an alkyl radical containing from 8 to 20 carbon atoms, and X is a halogen radical, and salts of such compounds to effect a substantially complete separation of the ore values from the acidic silicious gangue thereby producing a tailing high in phosphate and relatively low in gangue.

10 6. In the flotation process of separating acidic silicic gangue from phosphate ore values, the step which comprises subjecting the ore to froth flotation in the presence of an effective amount of unsymmetrical di-octyl guanidine hydrobromide to effect a substantially complete separation of the ore values from the acidic silicic gangue thereby producing a tailing high in phosphate and relatively low in gangue.

15

phate and relatively low in gangue.

7. In the flotation process of separating acidic silicious gangue from phosphate ore values, the 20 step which comprises subjecting the ore to froth flotation in the presence of an effective amount of lauryl biguanide hydrochloride to effect a substantially complete separation of the ore values from the acidic silicious gangue thereby producing 25 a tailing high in phosphate and relatively low in gangue.

30 8. In the flotation process of separating acidic silicious gangue from phosphate ore values, the step which comprises subjecting the ore to froth flotation in the presence of an effective amount of tetradecyl guanylurea hydrobromide to effect a substantially complete separation of the ore values from the acidic silicious gangue thereby producing a tailing high in phosphate and relatively low in gangue.

DAVID W. JAYNE, JR.  
HAROLD M. DAY.  
ELMER W. GIESEKE.